

June 8, 1937.

**F. J. CIRVES**

2,083,294

## PROCESS FOR BLEACHING PULP

Filed May 16, 1932



INVENTOR  
*Francis T. Cirves,*  
BY *Munn & Co.*

**ATTORNEY**

## UNITED STATES PATENT OFFICE

2,083,294

## PROCESS FOR BLEACHING PULP

Francis J. Cirves, Manistee, Mich.

Application May 16, 1932, Serial No. 611,692

2 Claims. (Cl. 8—2)

This invention relates to a process for bleaching pulp.

An object of the invention is the provision of a process for bleaching pulp such as wood, rag, 5 hemp, or other fibers by injecting free chlorine into an alkaline solution of the pulp.

A further object of the invention is the provision of a process for bleaching pulp in which an alkaline re-agent is thoroughly mixed with the 10 pulp and free chlorine is injected into the mixture at the point of greatest agitation.

A further object of the invention is the provision of a process for bleaching pulp in which an alkaline re-agent is mixed with the pulp and 15 during the beating action free chlorine is injected into the mixture at the point of greatest agitation for producing a nascent hypochlorite bleaching compound in direct contact with the fibers.

20 This invention will be best understood from a consideration of the following detailed description, in view of the accompanying drawing forming a part of the specification; nevertheless, it is to be understood that the invention is not confined to the disclosure, being susceptible of such 25 changes and modifications in which define no material departure from the salient features of the invention as expressed in the appended claims.

30 In the drawing:

Figure 1 is a horizontal section of a battery of beaters, and

Figure 2 is a vertical section of a bleacher showing the application of the free chlorine adjacent 35 the agitators or propellers.

Referring more particularly to Fig. 1 of the drawing, 10 designates a typical beater which is semi-circular at its ends in order to provide for the free circulation of the pulp. This type of 40 beater is provided with a bed plate (not shown) for the purpose of bringing the pulp in close association with the beater roll.

A feather 11 is located longitudinally of the container or vat 10 with its ends terminating 45 short of the semi-circular ends 12 of the container 10 so that there will be sufficient space to provide for the circulation of the pulp between the ends of the feather and the opposite ends of the container. It will be noted that this feature is hollow for a purpose which does not concern 50 the present invention.

A beater roll, generally designated by the numeral 13, is cylindrical in form and is secured to a shaft 14 driven by a pulley 15 from a suitable 55 source of power which uniformly drives the shaft 14 and the beater 13. It will be noted that the beater is provided with blades 16 which are adapted to come in contact with the fiber adjacent the bed plate in order that the fibers will be brushed

and hydrated and also circulated along the path indicated by the dotted lines 17 and 18.

A tank 20 is adapted to either contain chlorine gas or chlorine in the form of a liquid and the chlorine is conducted by a pipe 21 past a valve 22 to the branch pipes 23. A pipe or nozzle 24 located between the tank and the outer end of the branch pipe 23 is adapted to inject the chlorine into the mass within the container 10 at a point adjacent the beater roll 13 so that the chlorine will be injected into the mass at the point of greatest agitation. A valve 25 controls the flow of the chlorine to each container while the valve 22 controls the flow of the chlorine to the branch pipes 23.

Figure 2 is a vertical section of a type of pulp bleacher. This consists of a cylindrical tank 30 with a circular and sloping bottom 31 and 32. A top 33 forms a closure for the tank.

A pipe 34 enters the upper part of the tank 30 and provides means for supplying the tank 30 with the pulp. A pipe 35 is connected with the bottom of the tank and provides a discharge outlet for the pulp after it has been treated with an alkaline re-agent and bleached. A cylinder 36 is located centrally and vertically of the container 30. The opposite ends of the cylinder are open to provide for the inlet and discharge of the pulp.

A shaft 37 driven in any suitable manner (not shown) extends vertically and axially of the cylinder 36 and is provided with propellers 38 spaced at distances along the interior of the cylinder 36.

A pipe 39, which is formed preferably of hard rubber, extends through the top 33 and terminates at 40 within the cylinder 36 while the outer end 41 is connected with a tank for supplying the pipe with chlorine either in the form of a gas or liquid. A valve 42 controls the admission of the chlorine to the nozzle 40.

The top 33 is provided with an opening 43 through which the lime or soda is inserted for creating an alkaline condition of the pulp as will be presently explained.

It is to be understood that all of the parts of the device shown in Figs. 1 and 2 are formed of suitable material which will resist the action of the chlorine or certain parts may be formed of glazed tile or lined with a hard rubber coating or covered with a chlorine proof paint.

The operation of my device is as follows: The pulp is placed in the beaters and agitated in order to thoroughly break up the fibers and maintain them in a separated condition and an alkaline re-agent is supplied to the pulp at the proper time in an amount which approximates from 2% to 25% of the weight of the pulp. It will be appreciated that the amount of alkaline re-agent supplied will depend upon the type of pulp employed and the type of paper to be pro- 60

duced. This alkaline re-agent whenever referred to in the specification and claims is to be understood as being either an oxide or hydroxide or a carbonate of one of the four elements such as calcium, sodium, potassium, or magnesium.

The alkaline re-agent is thoroughly mixed with the pulp after which the valves that control the flow of the chlorine to the containers are opened, permitting the chlorine to be injected into the mixture or circulating mass at points of greatest agitation. In other words, the chlorine is injected at points adjacent the beater roll in any of the forms of the beaters which may be employed so that the chlorine is thoroughly mixed with the pulp and alkaline re-agent where it will act upon the alkaline re-agent and form a hypochlorite bleaching compound in a nascent state and thus the compound will be more effective to produce the proper degree of bleaching. These compounds are introduced directly into the pulp and may be used singly or in combination at varying percentages. As stated above from 2% to 25% of the alkaline bleach forming compounds to the weight of bone-dry stock are employed, the percentage depending upon the lightness of the bleach stock to be obtained. The alkaline compounds are introduced in dry or powdered form, or in solution, or in suspension with water. The free chlorine may be injected either in a gaseous or liquid form and the amount of chlorine varies from 2% to 25%, depending upon the degree of bleaching to be obtained. The chlorine may be introduced in a water solution.

The pulp is bleached at high or low consistency at any prescribed temperature or at any alkaline or pH control. The alkaline bleach forming the ingredients and chlorine are apportioned to produce the maximum effects of bleached qualities and physical strength characteristics, depending upon the variable conditions of consistency, temperature, alkaline pH and the kind of stock employed.

The bleaching process is especially adapted for the single stage, although several similar stages may be employed. The bleach or process is equally well adapted to the continuous or discontinuous or batch method.

In the discontinuous or batch method, the bleaching process is formed in a receptacle similar to a bleacher of several tons capacity, as shown in Fig. 2, which is regularly employed in the bleaching of pulp with the use of prepared hypochlorite bleaching solution. The bleacher should be concrete or stoneware or of other construction which is proof against the action of chlorine. The agitating propeller must be protected by rubber or other chlorine-proof covering or coating. The lime or soda is introduced into the bleaching receptacle with the stock and thoroughly mixed therewith. The chlorine is next introduced or injected, with agitation continuing thereafter until the bleaching is accomplished. The stock is then discharged and the device is ready for another batch.

From the above it will be seen that the process consists essentially of three steps which are combined for simultaneous operation: (1) the preparation of the hypochlorite bleach solution, (2) the pulp chlorinating process, and (3) the pulp bleaching process.

The chemical advantages of such simultaneous bleach operation are: (1) The intimacy of contact of the fibers and the reactive bleach forming constituents, (2) the increased activity of

bleaching agent upon the fibers which are chlorinated and immediately and directly exposed to bleaching, (3) the formation of nascent hypochlorite bleaching compound in contact with the fibers, (4) the beneficial action of agitation upon the simultaneous re-action of chlorination and oxidation, (5) the ease of bleaching at ordinary or low temperatures, (6) the beneficial color and strength effects obtained on the fiber, and (7) the rapidity, economy, and ease of obtaining a maximum bleach in one stage operation.

The use of hydrated lime and liquid chlorine is particularly well adapted to the above-described process of bleaching. The amount of lime incorporated in the pulp depends upon the degree of bleach desired and is practically 50% over the desired chlorine consumption. A specific instance for semi-bleaching will be approximated by 9% of hydrated lime and 6% of chlorine by weight to the bone-dry stock. This process is particularly adapted to the use of alkali thoroughly mixed with the pulp according to an established relationship between the desired chlorine consumption and the amount of alkali to be incorporated. This has been determined as approximately 1.5 to the weight of the chlorine to be consumed where the alkali used is hydrated lime or caustic soda. This enables proper control of the alkali, chlorine and the desired bleach. The process and the control may be employed in a single stage or similar multiple stages.

This process distinguishes from the other processes of pulp bleaching where the pulp is chlorinated in a general alkaline or non-alkaline stock or followed by an alkaline wash in the first stage and using hypochlorite bleach in the second stage.

Further processing or refinements in bleaching may be made with the above process but to obtain a desired whiteness or pH of bleached stock further treatment may be advisable. Alkali traces in the bleached product caused by impurities or otherwise may be counteracted with slight additions of dilute acids, such as hypochlorous acid, chlorine water, or a hypochlorite solution. Sulphuric acid, hydrochloric acid, or oxalic may be employed for counteracting the alkali traces.

I claim:

1. A process of bleaching pulp for the manufacture of paper which comprises thoroughly mixing fibrous pulp with hydrated lime and then injecting free liquid chlorine into the mixture of the pulp and lime while the mixture is being agitated, the quantity of chlorine injected being from two to twenty-five percent of the weight of the pulp, the approximate proportions of chlorine and lime being 1 to 1.5 so that an alkaline condition will be maintained during the bleaching action.

2. A process of bleaching pulp for the manufacture of paper which comprises beating fibrous pulp in a restricted space while maintaining circulation of the pulp, adding an alkaline re-agent to the pulp and thoroughly mixing the re-agent with the pulp by the beating action, and then injecting liquid chlorine into the mixture at a point where the pulp is being beaten so that the chlorine will be thoroughly mixed with the pulp and alkaline re-agent, the approximate proportions of chlorine and lime being 1 to 1.5 so that an alkaline condition will be maintained during the bleaching action.